

## UNITED STATES PATENT OFFICE

WILHELM KROLL, OF LUXEMBURG, LUXEMBURG

## PROCESS FOR THE PRODUCTION OF METALLIC BERYLLIUM

No Drawing. Application filed September 26, 1927, Serial No. 222,211, and in Germany September 28, 1926.

The present invention relates to a new useful process for the production of compact metallic beryllium.

Hitherto two kinds of processes have been used for the production of metallic beryllium, namely the chemical and the electrochemical processes.

In the chemical process beryllium chloride was reduced by an alkali metal. In this way spangles or scales of the metal are obtained which must be melted down into compact pieces in vacuo.

The only one of the electro-metallurgical processes which has been of any practical use is that one in which an electrolyte consisting of barium beryllium fluoride is subjected at about 1300° C. to electrolysis using cathodes which provide a good contact. By this process it is possible to obtain compact beryllium in comparatively large pieces. Unfortunately electrolysis requires a relatively large consumption of current and a considerable part of the beryllium is lost owing to the volatilization of the fluoride.

After thorough investigation of the conditions prevailing in the case of electrolysis I made the present invention according to which metallic beryllium can be obtained in a much simpler way by chemical decomposition. The reactions selected for the decomposition are based on the greater affinity of magnesium or of the earth alkali metals or of lithium for fluorine, so that beryllium fluoride can be decomposed in the simplest possible manner, and beryllium in the metallic form is set free. The decomposition reaction between the said metals and the beryllium fluoride is so violent that this reaction cannot be employed in practice owing to the great losses caused by volatilization. According to the present invention however the violence of the reaction can be damped down by diluting the beryllium fluoride with other salts, preferably with other fluorides. I have found it desirable to subject to such decomposing action, beryllium fluoride salt solutions free from water and diluted in the manner above described. The temperature during the new process is preferably at least about 1300° C. or somewhat higher. If it be desired to so con-

duct the reduction of the beryllium that beryllium completely free from any earth alkali metal, magnesium or lithium shall be obtained, provision must be made for a certain excess of beryllium fluoride or else the impure metallic beryllium obtained by the first decomposition must be decomposed again several times with fresh salt.

*Example.*—150 grams of  $MgF_2$ ,  $BeF_2$  were caused to react in a molten state with 20 grams of magnesium. The temperature rose above the melting point of beryllium so that compact metallic beryllium could be obtained. This however still contained about 5% of magnesium. By repeatedly decomposing the metallic beryllium obtained with 50 grams of the same salt I was able to obtain at 1300° C. perfectly pure metallic beryllium. If calcium be used for reduction, it is preferable to use calcium fluoride as the diluent for the beryllium fluoride. Metallic lithium which behaves similarly to the earth alkali metals may be used instead of magnesium or calcium for reduction but any alkali metal other than lithium cannot be used. On the other hand care must be taken to see that the molten mass contains only a little alkali fluoride as otherwise the reaction will be too violent and the alkali metal escapes in the form of vapour.

A number of other salts have been found to be satisfactory diluents for the beryllium fluoride such salts being preferably halogen compounds of the earth alkali metals. If such metallic salts be added to the mixture of salts, alloys of beryllium with the metal forming the base of these added salts will be formed. Thus for example aluminium-beryllium can be obtained by the decomposition of beryllium aluminium magnesium fluoride by metallic magnesium. By correctly selecting the salt components aluminium-beryllium alloys of high percentage and free from magnesium can be obtained. The same result is obtained if the metal with which the beryllium is to be alloyed be added to the bath not in the form of a metallic salt but in the form of any alloy with an earth alkali metal or as a pure metal. Thus aluminium-beryllium can be obtained from calcium-aluminium using beryllium fluoride as the reacting salt. Beryllium al-

loys of copper and iron are prepared in the same way.

The metallic beryllium obtained by the method above described can be purified or refined in a simple manner by superheating the crude beryllium obtained to free it from excess of earth alkali metal, the earth alkali metal being driven off in the form of vapour. This method is particularly easy to carry out in the case of magnesium-beryllium, which readily parts with its magnesium, if the temperature be raised to 1300° C. pure fused metallic beryllium remaining behind.

The carrying out of the process is however attended by difficulties in that the choice of suitable crucibles is a very restricted one. The earth alkali metals or the beryllium react with most of the substances which can be used and the fused fluorides assist the reaction to a very great extent. It was found that the reactions can be carried out in crucibles composed of fused alumina or magnesia or of beryllium oxide. It has however also been found of advantage to carry out the fusion in crucibles of pure graphite and to pour the fused mass into a vessel having water cooled walls and in which it is caused to react with magnesium or other earth alkali metals and can if necessary be kept hot by means of electrodes which provide a good contact. If the temperature be correctly selected and the composition of the mixture of salts is correct, the heat of combination of the magnesium with fluorine is sufficient to keep the reaction going and to raise the temperature to such a degree that compact fused metallic beryllium can be obtained.

In comparison with the electrolytic method the hereinbefore described chemical decomposition method possesses the great advantage that compact metallic beryllium is obtained in almost theoretical yield directly and in the shortest possible time and without any appreciable loss of beryllium fluoride.

Where in the appended claims I have mentioned an earth alkali metal, I desire this term to be interpreted as covering or including the equivalents mentioned above, that is to say, magnesium or lithium.

What I claim as my invention and desire to be secured by Letters Patent is:

1. The process for the production of compact metallic beryllium which consists in bringing to reaction fluorides of beryllium and at least one earth alkali metal free from water as a molten fused mass and at a temperature of at least about 1300° C., taking away the product of the reaction and melting it once more together with beryllium containing fluorides.

2. The process for the production of compact metallic beryllium which consists in bringing to reaction fluorides of beryllium and at least one earth alkali metal free from

water as a molten fused mass and at a temperature of at least about 1300° C., taking away the product of the reaction and melting it once more together with double fluorides of beryllium and of an earth alkali metal.

3. The process for the production of compact metallic beryllium which consists in bringing to reaction an excess of a beryllium fluoride compound free from water and at least one earth alkali metal, as a molten fused mass at a temperature of at least about 1300° C., taking away the product of the reaction and melting it once more together with beryllium containing fluorides.

In testimony whereof I affix my signature.

WILHELM KROLL.

70

75

80

85

90

95

100

105

110

115

120

125

130